

## UNITED STATES PATENT OFFICE

2,458,523

FROTH FLOTATION OF SULFIDE ORES IN  
THE PRESENCE OF A N-DICHLOROTHIO-  
CARBANILIDERutherford B. Martin, New York, N. Y., assignor  
to Kennecott Copper Corporation, New York,  
N. Y., a corporation of New YorkNo Drawing. Application October 5, 1945,  
Serial No. 620,648

3 Claims. (Cl. 209—166)

1

This invention relates to the concentration of ores and has for an object the provision of certain improvements in concentration operations. More particularly, the invention contemplates the provision of certain improvements in flotation operations. A further object of the invention is to provide certain improvements in flotation methods or processes.

The invention is based on my discovery that dichlorothiocarbanilide, represented by the following structural formula, is an effective flotation reagent:



Chlorinated thiocarbanilide may be prepared as follows: A mixture of 12 g. of m-chloroaniline with 10 c. c. of carbon disulphide was vigorously agitated with 10 c. c. of 40% sodium hydroxide. 20

10

15

20

2

The flotation reagent may be employed advantageously in neutral, alkaline and acid circuits. It may be employed advantageously in froth flotation operations designed for the concentration of both non-metallic minerals and metallic minerals and in froth flotation operations designed for the concentration of both oxidized ores and sulphide ores. The reagent can be employed with particular advantage in froth flotation operations designed for the concentration of sulphide ores.

The following examples illustrate the advantages of the reagent of the invention over reagents employed heretofore. The ore employed in the tests was Braden Copper Company ore containing on the average about 2.16% copper in sulphide form and about 0.21% copper in non-sulphide form and containing small amounts (about 0.075%) of molybdenite ( $\text{MoS}_2$ ). The ore was ground to 2.5% plus 100-mesh in all cases.

## Example 1

| Mineral Col-<br>lectors | Lb./ton<br>Req'd | Total<br>cost of<br>reagents<br>per ton<br>ore | Concts., per<br>cent |                | Tails, per<br>cent |                | Recoveries,<br>percent |                |
|-------------------------|------------------|------------------------------------------------|----------------------|----------------|--------------------|----------------|------------------------|----------------|
|                         |                  |                                                | Cu                   | $\text{MoS}_2$ | Cu                 | $\text{MoS}_2$ | Cu                     | $\text{MoS}_2$ |
| Standard.....           | .16              | .124                                           | 19.45                | .581           | .18                | .015           | 92.36                  | 81.28          |
| Standard.....           | .16              |                                                | 24.03                | .645           | .24                | .025           | 89.76                  | 69.76          |
| NaCl.....               | 1.80             | .148                                           | 13.70                | .560           | .11                | .019           | 95.72                  | 83.88          |
| Standard.....           | .16              |                                                | 24.15                | .644           | .22                | .025           | 90.64                  | 69.93          |
| NaCl.....               | 1.50             |                                                | 17.20                | .617           | .14                | .014           | 94.53                  | 86.10          |
| Kerosene.....           | .16              | .151                                           | 24.50                | .756           | .21                | .024           | 91.05                  | 69.56          |

## Example 2

| Mineral Col-<br>lectors           | Lb./ton<br>Req'd | Total<br>cost of<br>reagents<br>per ton<br>ore | Concts., per<br>cent |                | Tails, per<br>cent |                | Recoveries,<br>percent |                |
|-----------------------------------|------------------|------------------------------------------------|----------------------|----------------|--------------------|----------------|------------------------|----------------|
|                                   |                  |                                                | Cu                   | $\text{MoS}_2$ | Cu                 | $\text{MoS}_2$ | Cu                     | $\text{MoS}_2$ |
| Dichloro thio-<br>carbanilid..... | .10              | .071                                           | 18.60                | .650           | .14                | .022           | 94.40                  | 78.93          |
| Do.....                           | .10              |                                                | 24.80                | .750           | .42                | .028           | 82.43                  | 68.04          |
| NaCl.....                         | 1.50             | .095                                           | 18.70                | .611           | .13                | .015           | 94.75                  | 83.65          |
| Dichloro thio-<br>carbanilid..... | .10              |                                                | 24.40                | .617           | .30                | .028           | 87.58                  | 65.63          |
| NaCl.....                         | 1.50             |                                                | 17.75                | .638           | .15                | .016           | 94.05                  | 84.21          |
| Kerosene.....                     | .16              | .0976                                          | 24.15                | .789           | .25                | .020           | 89.37                  | 77.43          |

No solid was at first precipitated, but, after the addition of 20 c. c. of water and again shaking, 50 mm-dichlorothio-carbanilide was obtained in quantitative yield.

This method of preparing the compound is described in the Journal of the Society of Chemical Industry, vol. 45, 1926, page 351T.

The upper figures in the above tables indicate results obtained with Fagergren flotation machines, and the lower figures indicate results obtained with Minerals Separation flotation machines.

The standard reagent referred to in Example 1 55 is a well-known mineral collecting agent (ethyl

xanthogen ethylformate) accepted at the time of the tests as being the most effective in treating the ore tested, and the amounts indicated were the amounts considered to be most suitable.

I claim:

1. The method of concentrating sulphide ore which comprises subjecting the ore in the form of a pulp to a froth flotation operation in the presence of a chlorinated thiocarbanilide compound in which a chloride atom is attached to a nitrogen atom.

2. The method of concentrating sulphide ore which comprises subjecting the ore in the form of a pulp to a froth flotation operation in the presence of dichloro thiocarbanilide in which chlorine atoms are attached to nitrogen atoms.

3. The method of concentrating sulphide ore which comprises subjecting the ore in the form of a pulp to a froth flotation operation in the 20

presence of a compound having the following structural formula:



RHETHERFORD B. MARTIN.

#### REFERENCES CITED

10 The following references are of record in the file of this patent:

#### UNITED STATES PATENTS

| Number    | Name     | Date          |
|-----------|----------|---------------|
| 1,364,308 | Perkins  | Jan. 4, 1921  |
| 1,610,217 | Elley    | Dec. 7, 1926  |
| 2,061,243 | Lubs     | Nov. 17, 1936 |
| 2,106,552 | Jenkins  | Jan. 25, 1938 |
| 2,139,697 | Salzberg | Dec. 13, 1938 |
| 2,336,464 | Buck     | Dec. 14, 1933 |

**Certificate of Correction**

Patent No. 2,458,523.

January 11, 1949.

RHETHERFORD B. MARTIN

It is hereby certified that error appears in the printed specification of the above numbered patent requiring correction as follows:

Column 3, line 10, claim 1, for the word "chloride" read *chlorine*;  
and that the said Letters Patent should be read with this correction therein that the same may conform to the record of the case in the Patent Office.

Signed and sealed this 31st day of May, A. D. 1949.

[~~SEAL~~]

THOMAS F. MURPHY,  
*Assistant Commissioner of Patents.*